

# UNITED STATES PATENT OFFICE.

WILLIAM HENRY BRADSHAW, OF BROOKLYN, NEW YORK.

## PURIFIED GUM AND PROCESS OF OBTAINING SAME.

1,133,790.

Specification of Letters Patent. Patented Mar. 30, 1915.

No Drawing.

Application filed April 25, 1911. Serial No. 623,140.

*To all whom it may concern:*

Be it known that I, WILLIAM H. BRADSHAW, a citizen of the United States of America, residing in Brooklyn, in the 5 county of Kings and State of New York, have invented certain new and useful Improvements in Purified Gums and Processes of Obtaining Same, of which the following is a specification.

10 This invention relates to a process of purifying gums.

One of the objects of the present invention is to provide a simple and practical process of treating resin, gutta, Pontianak 15 and similar rubbery gums, or their constituents to remove impurities.

Another object is to provide an easy and inexpensive process of removing all objectionable tastes and principles from such 20 substances whereby they may be used in the arts.

Another object is to produce a purified ingredient used in the manufacture of chewing gum.

25 Other objects will be in part obvious and in part hereinafter pointed out.

The invention accordingly consists in the several steps and the relation and order of one or more of such steps with relation to 30 each of the others thereof which will be exemplified in the hereinafter described process, and the scope of the application of which will be indicated in the claims that follow.

35 As is well known to those familiar with the subject, chicle, a gum obtained from the latex of the sapota tree, and imported from Central American countries, forms an important ingredient in chewing gum. The

40 comparatively high cost of obtaining and subsequently purifying this substance has led to numerous attempts to produce a satisfactory substitute. Such a substitute has been found and principal ingredients there-

45 of consist of the purified waste product of deresinated rubber and also gutta, both essential parts of rubbery gums. Both of these substances contain either an objectionable taste, or some odor, and poisonous principles which it is necessary to remove before they can be used in the making of artificial chicle. It has been found that these may be removed by using sugar in solution.

Referring to the process more in detail, 50 the waste product of deresinated rubber may be treated as follows:—For example,

Pontianak resin, obtained as a by-product in deresinating Pontianak gum, sometimes called gutta jelutong, as sold, contains about 25% of moisture, dirt and particles of rubber. This is first partially dried and ground through an 8-mesh screen which removes the particles of rubber. The resin is then ground in water in a pebble mill in the presence of about 5% of sugar, if cane sugar is 60 used, although greater amounts may be used if desired. After grinding the resin in the mill until it will pass 60 to 100 mesh, it is diluted several times with water, boiled and filtered, and then washed with hot water 70 and then with cold water. The filter cake is then centrifuged and washed in a centrifugal machine and finally dried on trays in a drier.

The process of purifying gutta is quite 75 similar. It is first cut up and sorted to remove the larger particles of dirt, etc., and then placed in a hollander where it is reduced to very small particles. The gutta is then boiled in a 5% sugar solution substantially as above described, in order to remove any objectionable taste. The gutta is then removed and washed on ordinary rolls and hung up to dry.

As above stated, these rubber principles 80 form essential ingredients of a chicle substitute and when treated as above, are sufficiently pure and free from taste, odor and poisonous matters to be used freely as may be necessary.

It is thus seen that this invention provides a simple and practical process of purifying resins, guttas and similar gums in a quick and inexpensive manner.

As many changes could be made in carrying out the above process without departing from the scope of the invention, it is intended that all matter contained in the above description shall be interpreted as illustrative and not in a limiting sense.

I claim:

1. A process of treating gums which consists in treating resin element of a rubbery gum with sugar and thereby removing impurities therefrom.

2. A process of treating gums which consists in treating the resin element of a rubber gum with a solution of sugar and removing said sugar solution whereby impurities of said gum are eliminated.

3. A process of treating gums which consists in treating a rubber resin with a solu-

60

65

70

75

80

85

90

95

100

105

110

- tion of sugar heated to approximately 100° C., and thereafter removing the solution and impurities from said resin.
4. A process of treating gums which consists in treating resin occurring as a by-product gum in the deresination of Pontianak gum with sugar, whereby objectionable features are removed.
5. A process of treating gums which consists in treating resin occurring as a by-product gum in the deresination of Pontianak gum by a 5% cane sugar solution which is subsequently drawn off whereby objectionable features are removed.
- 15 6. A process of treating gums which consists in treating resin occurring as a by-product gum in the deresination of Pontianak gum by boiling the same in a sugar solution which is subsequently drawn off whereby objectionable features are removed.
- 20 7. A process of treating gums which con-

sists in treating gutta jelutong after reducing the same to small particles with a sugar solution whereby taste and poisonous matters are removed.

25

8. A process of treating gums which consists in reducing rubber gum to small particles, adding a sugar solution thereto, and after the particles become saturated, removing said solution, whereby the taste and 30 poisonous matters are eliminated.

9. A composition of matter the major portion of which is made from a rubber gum having a low per cent. of rubber and from which the rubber, taste and poisonous matters, which renders the composition objectionable as an ingredient of chewing gum are removed.

35 WILLIAM HENRY BRADSHAW.

Witnesses:

HAMILTON BRADSHAW,  
SAMUEL P. BRADSHAW.